# EUROPEAN PATENT SPECIFICATION

(11) **EP 2 152 947 B1**
(45) Date of publication and mention of the grant of the patent: **26.09.2012**
(21) Application number: 08734563.3
(22) Date of filing: 16.05.2008
(51) Int. Cl.: D04H 1/42, D04H 1/60

(54) **AN AIR-LAID NON-WOVEN FIBRE PRODUCT COMPRISING FIBRES OF RECYCLED MATERIAL**
TROCKENVLIESSTOFF MIT FASERN AUS REZYKLAT
PRODUIT FIBREUX NON TISSÉ FORMÉ PAR VOIE SÈCHE, COMPRENANT DES FIBRES DE MATÉRIAU RECYCLÉ

(30) Priority: 01.06.2007 DK 200700798
(43) Date of publication of application: 17.02.2010
(73) Proprietor: Formfiber Denmark APS, 8464 Skovby, Galten (DK)
(72) Inventor: ANDERSEN, Carsten, DK-8361 Hasselager (DK)
(74) Representative: Høiberg A/S
(86) International application number: PCT/DK2008/050108
(87) International publication number: WO 2008/145131

(56) References cited:
- WO-A-2005/044529
- DE-A1- 4 022 877
- US-A1- 2004 224 589
- US-A1- 2006 165 950

## Description

The present invention relates to air-laid non-woven fibre product manufactured by a dry forming process and a method of manufacturing such product.

From US-A-5,516,580 an insulation batt is known, where the material contains a portion of cellulose fibres, and longer bonding synthetic fibres. These synthetic fibres are so-called bi-component fibres that have an outer sheath which is heat-fused with outer sheaths of other synthetic fibres at crossing contact points thereof to form a matrix having pockets for retaining loose fill cellulose fibres therein. This matrix eliminates the need of an adhesive binder to retain the cellulose fibres in the matrix.

The drawback of this insulation board is that the fibre batt obtained hereby is not particularly resilient and the use of longer bi-component synthetic bonding fibres makes the product very expensive to manufacture.

A method of making a resilient mat is known from US-A-5,554,238. The insulation mat according to this method comprises cellulosic and thermoplastic fibres. A mat is formed in an air-laying process and subsequently the surface is flame-treated to melt the thermoplastic component on the surface forming a skin which keeps the cellulosic fibres intact. The thermoplastic fibres in the interior of the mat remains unmelted, whereby the mat is provided with a spring-back characteristic, which allows the mat to retain most of its original shape after it has been compressed, e.g. for shipping.

However, this resilient mat has a "crisp" exterior surface reducing the resiliency of the mat as a whole and not homogeneously bonded throughout the product, which does not allow for easy handling since the product may easily delaminate or otherwise break up. The insulation effect is moreover reduced due to the more compact structure of the fibre product.

From WO 01/48330 a recyclable insulating mat comprising shredded waste paper or cardboard mixed with natural fibres and 5-50 % polyester is known.

In DE 196 02 551 C1, there is described a mat for manufacturing self-supporting form parts by heat treatment. The mat comprises long natural fibres and thermoplastic binding means provided as synthetic fibres. The thermoplastic binding means are provided synthetic material with a high melting point and a low melting point.

A method for creating a wood-substitute material comprising recycled synthetic fibers is known from US 2004/0224589 A1.

It is an object of the present invention to provide a resilient fibrous product which is recyclable and inexpensive to manufacture from waste material.

This object is achieved by an air-laid non-woven fibre product as defined in claim 1.

According to a second aspect of the invention, there is provided a method of manufacturing a non-woven product as defined in claim 8.

According to the invention, an air-laid fibrous product is obtained based on recycled fibres from waste material from recycled tires. These tires are among the largest and most problematic sources of waste, due to the large volume produced and their durability. Those same characteristics which make waste tires such a problem also make them one of the most re-used waste materials, as the rubber is very resilient and can be reused in other products. Thus, the rubber of the scrap tires may be recycled, but by the present invention, it is realised that also the other material components of the scrap tires may be recycled.

When a scrap tire is to be recycled, the tires are shredded and the rubber components are separated from the rest of the waste material and collected for reuse in other products. However, the remaining waste material comprising shredded textile material cannot be recycled. This waste tires textile material also contains residues of rubber and metal wires.

By the invention, it is realised that the shredded tires fabric material can be recycled in an advantageous manner by utilising this material in an air-laid fibre mat which is obtainable by using the manufacturing technology disclosed in WO2005/044529.
The fibre mat product according to the invention is furthermore advantageous since the product is water repellent and provided with resilience whereby the mat raises again after compression and resumes its original shape.

This advantageous characteristic of the product according to the invention is also achieved by the use of short bi-component fibres so that the resulting fibrous mat is very flexible as the short bi-component fibres acting as binding means in the product are short. The bi-co fibres become hard when cured after having been heated above the melt temperature, so by using short bi-co fibres the bi-co fibres do not adversely affect the resulting product with respect to flexibility and elastic properties when cured due to their short length.

Moreover, it is realised by the invention that the short bi-component fibres mix better with the recycled fibres whereby a substantially small proportion of bi-co fibres are needed to provide sufficient coherence of the product. This further enhances the flexibility of the fibrous product.

In a preferred composition of the fibre product, 80-90 % recycled shredded tire material fibres are used together with 10-20 % bonding fibres. The bonding fibres are bi-component fibres substituted or supplemented with polyester fibres, polypropylene and/or other plastic fibres having bonding characteristics.

The product according to the invention is found particularly advantageous since it is flexible and whether and water resistant and may thereby substitute e.g. foam sheets in the building industry. Other useful purposes may be vibration or noise damping, e.g. of wooden floors, use in noise screens in road constructions, etc.

Preferably, the fibre length of the shredded material in the first portion is 1-100 mm, and the grammar weight of the air-laid product according to the invention is between 20 kg/m³ and 200 kg/m³.

In an embodiment of the invention, addition fibres, such as recycled glass fibres, carbon fibres or the like, may be added to the first portion.

At least 50 % of the bi-component fibres are crimped fibres with a length between 2 to 50 mm. By using short and crimped fibres, e.g. of a helical shape extra flexibility and resilience is achieved in the product allowing the product to appear softer and having good properties with respect to raising again after compression and resuming its original shape.

In a preferred embodiment, the fibres are provided with fire-retarding chemical, such as Borax, Boric acid, Ammonium sulphate or aluminium sulphate, mixed with the fibres, e.g. in the forming box before being laid on the forming wire. In another embodiment, the dry-formed fibre mat may be sprayed with fire-retarding chemical, e.g. after the mat is formed and heated.

If extra bonding of the fibres is required, an additional fluidized binder may be sprayed into the forming box and onto the fibres therein. The fluidized binder may alternatively be sprayed onto the fibres. As a further alternative or as a supplement, binder in pulverised form may be mixed with the fibres before the mixture is forwarded to the forming box.

The invention is further explained with reference to the accompanying drawing which shows a diagram of an embodiment of the manufacturing process for producing a product according to the invention.

Waste material from shredded tires mainly consisting of tire fabric shredded into fibres in a length below 100 mm. Although mainly consisting of fabric from the tires, the shredded waste fibres also contain residues of rubber and some pieces of metal wire which have not been recovered from the shredded tire material for immediate reuse.

This shredded fabric fibre material including residue material constitutes a first fibre portion which is mixed with bi-component fibres. These bi-component fibres comprise a core and an outer sheathing, said outer sheathing having a first melting temperature which is lower than the second melting temperature of the core. The purpose these bi-component fibres serve is to provide bonding between the fibres in the first portion of fibres. The bi-component fibres become hard when cured after having been heated above the melt temperature, so by using short bi-co fibres the bi-co fibres do not adversely affect the resulting product with respect to flexibility and elastic properties when cured due to their short length. Moreover, the short bi-component fibres blend very well with the fibres of the first portion ensuring a more homogeneous bonding throughout the product.

The mixture of fibres are forwarded to a forming box, preferably of the kind described in WO2005/044529, where the box is provided with a revolving belt screen allowing for an even distribution of fibres irrespective of their size.

The fibres are introduced into the forming box and laid on the forming wire beneath the forming box. The web of fibres is forwarded in a continuous motion through a heating station where the bi-component fibres are activated and the fibrous web is provided with its coherence.

The web is then cured as the heated bi-component fibres are cooled and the web may be forwarded through a pressing station for providing the resulting mat product with a predetermined density.

The fibrous web may be sprayed with a fire-retarding substance, such as Borax, Boric acid, Ammonium sulphate or aluminium sulphate, for providing the product with fire-retarding properties. Alternative to spraying the formed web, this substance could also be sprayed into the forming box and thereby priming the fibres before the fibres are laid onto the forming wire.

### Example:

### Example I:

A material for forming an insulation fibre mat is mixed by provided the following components:
90 % shredded scrap tire fabric fibres of recycled tires.
10 % bi-component fibres of approx. 6 mm length having a coated polyester core.

The fibres are laid by the forming box and heated to a temperature of 130°C and then primed with a fire retardant.

Hereby, a cost effective fibre product having a grammar weight of 20-200 kg/m³ is provided, which has a good spring elastic effect and insulation properties.

By the present invention, it is realised that the variations of the above-mentioned example may be performed without departing from the scope of the invention as defined in the accompanying claims.

## Claims

1. An air-laid non-woven fibre product manufactured by a dry forming process, said product comprising:
a first portion of up to 98 % recycled shredded material, where the shredded material is a mixture of shredded fabric material fibres from automotive tires or
the like and residues of rubber and other components from the shredded tires, and
a second portion of 1 - 30 %, preferably 1 - 5 %, bi-component fibres having a length between 2 - 50 mm, preferably 2-6 mm in length, and comprising a core and an outer sheathing, said outer sheathing having a first melting temperature which is lower than the second melting temperature of the core and that at least a major portion of the bi-component fibres are crimped fibres.

2. A product according to claim 1, wherein the fibre length of the shredded material in the first portion is 1-100 mm.

3. A product according to any of the preceding claims, wherein addition fibres, such as recycled glass fibres, carbon fibres or the like, may be added to the first portion.

4. A product according to any of the preceding claims, wherein the fibres are provided with fire-retarding chemical, such as Borax, Boric acid, Ammonium sulphate or aluminium sulphate, mixed with the fibres.

5. A product according to any of the preceding claims, wherein the dry-formed fibre mat is sprayed with fire-retarding chemical.

6. A product according to any of the preceding claims, wherein the gram weight of the air-laid product is between 20 kg/m³ and 200 kg/m³.

7. A product according to any of the preceding claims, wherein the first portion comprises 80-90 % by weight and the second portion comprises 10-20 % by weight of the total fibre composition.

8. A method of manufacturing a non-woven product of the kind mentioned in claims 1 to 7 by dry forming a product of fibrous material, said method comprising the steps of:
advancing fibrous material into a forming box having a bottom outlet positioned over a forming wire to form a web of dry-laid fibres on the forming wire, where said fibrous material comprises
a first portion of up to 98 % recycled shredded material, where the shredded material is a mixture of shredded fabric material fibres from automotive tires and residues of rubber and other components from the shredded tires, and
a second portion of 1 - 30 %, preferably 1 - 5 %, bi-component fibres with a length between 2 - 50 mm and comprising a core and an outer sheathing, said outer sheathing having a first melting temperature which is lower than the second melting temperature of the core and wherein at least a major portion of the bi-component fibres are crimped fibres;
heating the web of fibres formed on the forming wire to a temperature above the first melting temperature; and
advancing the fibrous web through a pressing section whereby a fibrous product web with a predetermined density is formed.

9. A method according to claim 8, whereby a fluidized binder is sprayed into the forming box and onto the fibres therein.

## Patentansprüche

1. Airlaid-Faservlies-Produkt, hergestellt mittels eines Trockenform-Verfahrens, welches umfasst:
einen ersten Anteil von bis zu 98 % aus rezykliertem geschredderten Material, worin das geschredderte Material ein Gemisch von geschredderten Gewebematerial-Fasern aus Kraftfahrzeugreifen und Resten von Gummi und anderen Komponenten der geschredderten Reifen ist, und
einen zweiten Anteil von 1 - 30 %, vorzugsweise 1 - 5 % Zweikomponenten-Fasern mit einer Länge zwischen 2 - 50 mm, vorzugsweise 2 - 6 mm und einem Kern und einer äusseren Umhüllung, wobei die äussere Umhüllung eine erste Schmelztemperatur aufweist, die unter der zweiten Schmelztemperatur des Kerns liegt, und worin mindestens ein grösserer Teil der Zweikomponenten-Fasern gefaltete Fasern sind.

2. Produkt nach Anspruch 1, worin die Faserlänge des geschredderten Materials in dem ersten Anteil 1 - 100 mm beträgt.

3. Produkt nach einem der vorstehenden Ansprüche, worin zusätzliche Fasern, wie rezyklierte Glasfasern, Carbonfasern oder dergleichen zu dem ersten Anteil zugesetzt werden können.

4. Produkt nach einem der vorstehenden Ansprüche, worin die Fasern mit einer flammhemmenden Chemikalie, wie Borax, Borsäure, Ammoniumsulphat oder Aluminiumsulphat bereitgestellt werden, die mit den Fasern vermischt ist.

5. Produkt nach einem der vorstehenden Ansprüche, worin die trockengeformte FaserMatte mit der flammhemmenden Chemikalie besprüht ist.

6. Produkt nach einem der vorstehenden Ansprüche, worin das Gramm-Gewicht des Airlaid-Produkts zwischen 20 Kg/m³ und 200 kg/m³ liegt.

7. Produkt nach einem der vorstehenden Ansprüche, worin der erste Anteil 80 - 90 Gew.-% und der zweite Anteil 10-20 Gew.-% der Gesamt-Faserzusammensetzung umfasst.

8. Verfahren zur Herstellung eines Faservlies-Produkts nach einem der Ansprüche 1 bis 7 durch Trockenformen eines Produkts eines faserförmigen Materials, welches die Schritte umfasst:
Vortreiben eines faserförmigen Materials in einen Formbehälter mit einem Auslass am Boden, das über einem Formband angeordnet ist, um ein Gewebe aus trockengeformten Fasern auf dem Formband zu bilden, wobei das Faser-Material umfasst,
einen ersten Anteil von bis zu 98 % aus rezykliertem geschreddertem Material, worin das geschredderte Material ein Gemisch von geschredderten Gewebematerial-Fasern aus Kraftfahrzeugreifen und Resten von Gummi und anderen Komponenten der geschredderten Reifen ist, und
einen zweiten Anteil von 1 - 30 %, vorzugsweise 1 - 5 % aus Zweikomponenten-Fasern mit einer Länge zwischen 2 - 50 mm und einem Kern und einer äusseren Umhüllung, wobei die äussere Umhüllung eine erste Schmelztemperatur aufweist, die unter der zweiten Schmelztemperatur des Kerns liegt, und worin mindestens ein grösserer Teil der Zweikomponenten-Fasern gefaltete Fasern sind;
Erhitzen des auf dem Formband gebildeten Gewebes der Fasern auf eine Temperatur über der ersten Schmelztemperatur; und
Vortreiben des Fasergewebes durch einen Pressbereich, wobei ein faserförmiges Gewebeprodukt mit einer bestimmten Dichte gebildet wird.

9. Verfahren nach Anspruch 8, wobei ein fluidisierter Binder in den Formbehälter und auf die darin befindlichen Fasern gesprüht wird.

## Revendications

1. Produit de fibres non tissées formé par voie sèche fabriqué par un procédé de formation par voie sèche, ledit produit comprenant :
une première portion allant jusqu'à 98 % de matériau déchiqueté recyclé, où le matériau déchiqueté est un mélange de fibres de matériau d'étoffe déchiqueté provenant de pneus automobiles et de résidus de caoutchouc et d'autres composants issus de pneus déchiquetés, et
une seconde portion allant de 1 à 30 %, de préférence de 1 à 5 % de fibres à deux composants ayant une longueur entre 2 et 50 mm, de préférence entre 2 et 6 mm de longueur, et comprenant une âme et une gaine externe, ladite gaine externe ayant une première température de fusion qui est inférieure à la seconde température de fusion de l'âme et au moins une portion majeure des fibres à deux composants étant des fibres crêpées.

2. Produit selon la revendication 1, dans lequel la longueur de fibre du matériau déchiqueté dans la première portion est de 1 à 100 mm.

3. Produit selon l'une quelconque des revendications précédentes, dans lequel des fibres d'addition, telles que des fibres de verre recyclées, des fibres de carbone ou similaire, peuvent être ajoutées à la première portion.

4. Produit selon l'une quelconque des revendications précédentes, dans lequel les fibres sont dotées d'un produit chimique ignifuge tel que le Borax, l'acide borique, le sulfate d'ammonium ou le sulfate d'aluminium, mélangé avec les fibres.

5. Produit selon l'une quelconque des revendications précédentes, dans lequel le produit chimique ignifuge est pulvérisé sur le mat de fibres formé par voie sèche.

6. Procédé selon l'une quelconque des revendications précédentes, dans lequel le poids en grammes du produit formé par voie sèche est compris entre 20 kg/m³ et 200 kg/m³.

7. Produit selon l'une quelconque des revendications précédentes, dans lequel la première portion comprend 80 à 90 % en poids et la seconde portion comprend 10 à 20 % en poids de la composition de fibres dans sa totalité.

8. Procédé de fabrication d'un produit non tissé de type mentionné dans les revendications 1 à 7 par formation par voie sèche d'un produit de matériau fibreux, ledit procédé comprenant les étapes consistant à :
faire avancer le matériau fibreux dans une boîte de formation ayant un refoulement inférieur positionné sur une toile de formation afin de former un voile de fibres formées par voie sèche sur la toile de formation, où ledit matériau fibreux comprend
- une première portion allant jusqu'à 98 % de matériau déchiqueté recyclé, où le matériau déchiqueté est un mélange de fibres de matériau d'étoffe déchiqueté provenant de pneus automobiles et de résidus de caoutchouc et d'autres composants issus de pneus déchiquetés, et
- une seconde portion de 1 à 30 %, de préférence de 1 à 5 % de fibres à deux composants d'une longueur allant de 2 à 50 mm et comprenant une âme et une gaine externe, ladite gaine externe ayant une première température de fusion qui est inférieure à la seconde température de fusion de l'âme et dans lequel au moins une portion majeure des fibres à deux composants est des fibres crêpées ;
chauffer le voile de fibres formé sur la toile de formation à une température supérieure à la première température de fusion ; et
faire avancer le voile fibreux à travers une section de pressage, un voile de produit fibreux d'une densité prédéterminée étant ainsi formé.

9. Procédé selon la revendication 8, un liant fluidisé étant ainsi pulvérisé dans la boîte de formation et sur les fibres qui se trouvent à l'intérieur de celle-ci.
